# EUROPEAN PATENT SPECIFICATION

(11) **EP 0 512 994 B1**
(45) Date of publication and mention of the grant of the patent: **15.11.1995**
(21) Application number: 90914553.4
(22) Date of filing: 01.10.1990
(51) Int. Cl.: D04C 1/06

(54) **ABRASION RESISTANT BRAIDED SLEEVE**
VERSCHLEISSFESTER GEFLOCHTENER SCHLAUCH
GAINE TRESSEE RESISTANTE A L'ABRASION

(43) Date of publication of application: 19.11.1992
(73) Proprietor: THE BENTLEY-HARRIS MANUFACTURING CO., Lionville, Pennsylvania 19353 (US); T&N PLC, Manchester M17 1RA (GB)
(72) Inventor: GLADFELTER, Harry, Foster, Phoenixville, PA 19460 (US)
(74) Representative: Crux, John Anthony
(86) International application number: GB9001498
(87) International publication number: WO9206235

(56) References cited:
- EP-A- 0 117 057
- EP-A- 0 134 864
- EP-A- 0 249 333
- DE-A- 3 344 866

## Description

This invention relates to braided products in general and in particular to braided tubular sleeving which can be placed over various substrates such as wire bundles, pipes, conduits, electrical cables, air hoses and the like to provide abrasion resistance and improved appearance.

### Background of the Invention

Some substrates such as electrical wire or cable are overbraided with wire to provide electrical shielding and other substrates such as hydraulic hoses are overbraided with wire or other materials to provide increased strength characteristics. In both instances the overbraiding can also provide increased abrasion resistance and durability for the product. However, in many instances it is impractical to overbraid such substrates with a desired exterior material. For example, electrical wires and cables are frequently installed in computer installations and particularly in robotic installations wherein it is desirable to bundle a number of wires or cables together and retrofit a flexible sleeving over the wire or cable bundle at the time of installation or some time after the original installation. In other circumstances it is desirable to protect other conduits such as air, water or other hoses by retrofitting sleeving over the hose at the time or installation or thereafter.

It is known from DE-A-3344866 to make self-supporting tubes of braided monofilaments with additional threads for increased rigidity.

Braided tubular sleeving has conventionally been used as field installed protective sleeving. One such product is the EXPANDO self-fitting protective oversleeve made by Bentley-Harris Manufacturing Co., Lionville, Pennsylvania. The EXPANDO sleeving is a braided tubular product made from a resilient engineering plastic yarn such a monofilament polyester. The EXPANDO oversleeve is particularly well suited for field installation over wire and cable bundles or harnesses, hoses, and the like because the sleeving material has an open weave construction which enables the braided tube to expand three times its original diameter when the braided tube is axially compressed. When the axial compression is released the braided tube tends to return to its original smaller diameter due to the resilient nature of the engineering plastic yarn from which it is braided. This "springback" property gives the braided sleeving the desirable characteristic of being self-fitting and conforming to any size substrate which is larger than the original diameter of the sleeve and to any irregular shape of wire and cable bundle. Once installed on the substrate the braided sleeving tends to remain tightly conformed to the exterior of the substrate. Since the braided open weave construction of the oversleeving is very flexible, the oversleeving easily conforms during any bending and flexing of the substrate thus providing continual protection for the substrate.

### Summary of the invention

According to the present invention, a field installable flexible tubular sleeve comprises braided, resilient strands, wherein each resilient strand is comprised of 1 to 10 monofilaments of an engineering plastic material having a modulus of elasticity of at least 3860 MN/m² (500,000 psi), said braided resilient strands defining a plurality of pair of cross over points within said sleeve, said braided sleeve further comprising uniformly distributed, flexible and substantially nonresilient relatively limp warp yarns interthreaded into said braid, said sleeve having at least a first and a second position, whereby:
a portion of said braided, resilient strands in said first position are longitudinally compressed and radially expanded and said limp warp yarns tend to uniformly form very small loops between each of the pairs of cross over points where said warp yarns are located in said longitudinally compressed and radially expanded portion of said braided resilient strands; and in said second position, said portion of said braided resilient strand is longitudinally extended and radially compressed, and said limp warp yarns are substantially straightened so as to substantially retract said loops.

The preferred resilient yarn comprises polyester and the preferred warp yarn comprises any limp, nonresilient natural or synthetic multifilament yarn and may be a texturised or spun yarn. Within these broad parameters, the particular warp yarn chosen will be dependent upon the desired end purpose.

An important objective of the invention is the provision of abrasion resistant braided sleeves which have improved coverage and tensile strength properties without sacrifice of the desirable springback of such sleeves.

A still further object of the invention is the use of warp yarns in a braided resilient sleeve for longitudinal stiffness, coverage and dimensional stability, without impairment of the pushback and springback capability of the braided tubular structure.

A still further object of the invention is the provision of warp yarns in a braided sleeve in which the warp yarns are constructed so as to eliminate the tendency to loop and snag as the braided structure is expanded and then contracted.

### General Description of the Drawings

Figure 1 shows a braided sleeve according to the present invention; and
Figure 2 shows a fragmentary view on an enlarged scale, schematically illustrating the construction of the sleeve of Figure 1.

### Description of the Invention

Although flat braiding techniques may be employed, the braided products formed by the teachings of this invention may be fabricated using conventional circular braiding equipment. As is recognized in the art, a circular braider is provided with a ring of studs distributed in uniformly spaced relationship around the braider with each stud receiving a spool of strand or yarn. Movement of the spools in sinuous paths produces a braided sleeve of selected properties in a manner known to those of ordinary skill in the art.

In carrying out the invention, spools of engineered plastic monofilament strand each comprised of 1 to about 10 monofilaments are uniformly distributed on the ring of studs. Additional studs between the studs for supporting the spools of monofilament strand are provided for the support of spools for the warp yarns utilized in the present invention. In accordance with the conventional techniques, known to those of ordinary skill in the art, the braider is used to form an open weave braid which is highly flexible and radially expandable to facilitate installation over wire bundles or hoses which may have irregularly shaped connectors or fittings attached. The facility of radially expanding and contracting allows the sleeving to snugly and neatly conform to irregularities in the profile of the cable bundle or hose.

The resilient engineered plastic strand useful in this invention should have sufficient tensile modulus to provide the desired springback characteristic in the braided sleeving. Preferably, the strand used is polyester but it will be appreciated that any of the family of plastics known as engineered plastics are suitable for use in the sleeves of this invention. By resilient engineered plastics, it is meant that the plastic has a tensile modulus of greater than 689MN/m² (100,000 psi) and preferably greater than 1034 MN/m² (150,000 psi) and more preferably at least 2068 MN/m² (300,000 psi). Examples of engineered plastics are the olefin polymers, of which some preferred olefin polymers are high density polyethylene, polypropylene, polybutene-1, poly 4-methyl pentene and fluorinated polyolefins such as ethylenetrifluorochloroethylene copolyers, ethylenetetrafluoroethylene copolymers, and vinylidene fluoride polymers, especially polyvinylidene fluoride, and blends thereof, for example, the fluorinated olefin blends as described in British patent No.1 1,120,131; polyesters, for example, polyethylene terephthalate, polytetramethylene terephthalate for example those treated as described in U.S. patent Nos. 3,968,015; 4,073,830 and 4,113,594; polyphenylene-oxide and -sulphide, blends of polyethylene oxide with polystyrene, silicone-carbonate block copolymers, polyketones, such as polyarylether ketones, for example, those described in U.S. patent Nos. 3,953,400; 4,024,314; 4,229,564; 3,751,398; 3,914,298; 3,965,146; and 4,111,908; polysulphones, for example, polyaryl sulphones, polyarylether sulphones, polyetherimides, for example those described in U.S. patent No. 3,847,867, polycarbonates especially those derived from bis phenol-A, polyamides, especially those described in U.S. patent No. 3,551,200 and 3,677,921, epoxy resins and blends of one or more the above-mentioned polymeric materials either with each other or with other polymeric materials. Additional discussion of such materials is found in British specification No. 1,529,351. The disclosure of the above patents and specifications are incorporated herein by reference.

Although other monofilament yarns or strands may be employed, in forming a one inch internal diameter sleeve, polyester monofilament strands having a diameter of about 10 mils such as are available under the trade mark ESTRALYN from Johnson Filament of Williston, Vermont are provided in strand form wherein each strand is comprised of three monofilament ends. The strands are loaded on each of 48 carriers on the braider and are braided to form a sleeve of open weave construction.

A braided sleeve so formed has excellent pushback and springback characteristics so that it readily and easily is made to fit over elongated substrates and is easily radially expanded and contracted so as to snugly fit over regular surfaces.

In carrying out the objectives of the present invention a sleeve of the type described is modified by the addition of relatively limp multifilament warp yarns. These warp yarns are preferably spun or texturised yarns. Other yarns may be employed provided that they meet the requirement of being relatively limp. Such yarns may be formed from either natural or synthetic fibres, the synthetic fibres being either organic or inorganic fibres. For applications where it is desirable to increase the density and reduce the permeability of the braided structure, bulkier warp yarns may be employed. For applications where the warp yarns are to be provided to increase the tensile strength of the product, as for example wiring harnesses, where the sleeve provides strain relief, less bulky yarns, characterized by their tensile properties will be employed. Likewise the number of warp yarns in relation to the monofilament strands will be dependent upon the end use of the particular product. In conventional braiding equipment, an extra stud is provided between each braider bobbin stud and this stud may be utilized for a spool of warp yarn. Thus, bobbins of warp yarn may be provided between every other braid strand bobbin for a product having maximum coverage and good pushback and springback. Where stability or strain relief are the primary requirements, the ratio of warp yarns to monofilaments may vary substantially depending upon the desired properties and the tensile strangth of the warp yarns, For example, an end product of open braid construction, where it is desirable to increase the structural stability of the product and provide strain relief while retaining the open construction to allow for air flow, may have warp yarns present in a ratio of 1 to about 2 to 4 braided monofilament strands. This can be accomplished by placing the spools of warp yarns between the appropriate groups of spools of braid strands. A sleeve 10 formed in accordance with the invention is shown in Figures 1 and 2. The sleeve comprises strands 11 and 12, each comprised of 3 monofilament ends. Warp yarns 13 extend lengthwise of the sleeve.

In use of a sleeve formed in accordance with the invention, when the sleeve is pushed back and radially expanded, the relatively limp warp yarns compress and tend to uniformly form very small loops between each of the cross over points in the braided structure. When the braided structure is allowed to springback, the warp yarns return to their original straightened condition within the structure so that none of these loops remain. In contrast, when warp yarns or strands of monofilament are utilized to give the structure body, these warp monofilaments slip relatively to the braided strands and tend to buckle at irregular intervals producing relatively large loops or kinks at the points where buckling takes place. When the braided structure springs back to its original configuration, these loops, commonly called "loopies" by those working in this art, remain. These loopies not only detract from the appearance of the sleeve, they greatly impair the function since they are easily snagged and broken and are targets for abrasion. Ultimately, they lead to kinks and holes in the harness, destroying its usefulness. In contrast, the multifilament yarns add strain relief, coverage and stability to the braided product without the disadvantage caused by the monofilament loopies.

If desired, the multifilament warp yarns of the invention may be comprised of filaments coated with a heat activatable adhesive. Sleeves so formed would have the properties of a braided sleeve during installation. Once in place, particularly in applications where abrasion from vibration or movement is a problem, the adhesive is activated to permanently lock the structure in place.

As indicated above, the warp yarns may be added in a similar fashion to flat braided monofilament sheets. The multifilament warp yarns substantially eliminate the fishnet characteristic of tapes or sheets made entirely of monofilament yarns and eliminate the tendency to form "loopies" as well as the stiffness imparted to such a braided structure when monofilament warp yarns are included.

### Example

A one inch internal diameter sleeve was braided using a 96 carrier circular braider from strand comprised of three ends of 10 mil monofilament polyester available under the trade mark ESTRALYN sold by Johnson Filament of Williston, Vermont. This material has a modulus of elasticity of 750,000 psi. Between every 7 carriers there was provided a carrier of texturised warp yarn of 1,000 denier multifilament nylon available under the trade mark CORDURA sold by E.L. DuPont De Nemours. This warp yarn is a relatively limp yarn imparted to the braided sleeve improved body and coverage, without impairment of its springback characteristics.

## Claims

1. A field installable flexible tubular sleeve comprising braided, resilient strands, wherein each resilient strand is comprised of 1 to 10 monofilaments of an engineering plastic material having a modulus of elasticity of at least 3447MN/m² (500,000 psi), said braided resilient strands defining a plurality of pair of cross over points within said sleeve, said braided sleeve further comprising uniformly distributed, flexible and substantially nonresilient relatively limp warp yarns interthreaded into said braid, said sleeve having at least a first and a second position, whereby:
a portion of said braided, resilient strands in said first position are longitudinally compressed and radially expanded and said limp warp yarns tend to uniformly form very small loops between each of the pairs of cross over points where said warp yarns are located in said longitudinally compressed and radially expanded portion of said braided resilient strands; and
in said second position, said portion of said braided resilient strand is longitudinally extended and radially compressed, and said limp warp yarns are substantially straightened so as to substantially retract said loops.

2. A sleeve according to claim 1, comprising one warp yarn for every 1-4 monofilaments.

3. A sleeve according to claim 1, comprising about one warp yarn for every 2 resilient strands.

4. A sleeve according to claim 3, wherein the monofilaments are a polyester.

5. A sleeve according to claim 4, wherein the monofilaments have a diameter of 0.15 to 0.375mm (6 mils to 15 mils).

6. A braided structure according to claim 5 wherein said resilient strand comprises from about 2 to about 6 ends of polyester monofilament having a diameter of about 0.15 to 0.375 mm (6 to about 15 mils) and a modulus of elasticity of about 5171 MN/m² (750,000 psi).

## Patentansprüche

1. Vor Ort einbaubarer, flexibler, rohrförmiger Schlauch umfassend geflochtene, elastische Litzen, worin jede elastische Litze aus 1 bis 10 Einzelfäden aus einem technischen Kunststoffmaterial besteht, welches einen Elastizitätsmodul von wenigstens 3447 MN/m² (500.000 psi) aufweist, welche geflochtenen, elastischen Litzen eine Mehrzahl von Paaren von Überkreuzungspunkten in diesem Schlauch bilden, wobei der geflochtene Schlauch weiters gleichmäßig verteilte, flexible und im wesentlichen nicht-elastische, relativ biegsame Kettgarne in diesen Schlauch eingeflochten aufweist, welcher Schlauch wenigstens eine erste und eine zweite Position aufweist, worin:
ein Abschnitt der geflochtenen, elastischen Litzen in dieser ersten Position in Längsrichtung gepreßt und radial aufgeweitet vorliegt und die biegsamen Kettgarne dazu tendieren, gleichmäßig sehr kleine Schlingen zwischen jedem Paar von Überkreuzungspunkten auszubilden, wo die Kettgarne in diesem in Längsrichtung gepreßten und radial aufgeweiteten Bereich der geflochtenen, elastischen Litzen angeordnet sind; und
in der zweiten Position dieser Abschnitt der geflochtenen, elastischen Litzen in Längsrichtung gedehnt und radial gepreßt vorliegt und die biegsamen Kettgarne im wesentlichen gestreckt ausgebildet sind, um die Schlingen im wesentlichen zuzuziehen.

2. Schlauch nach Anspruch 1, umfassend ein Kettgarn für jeweils 1-4 Einzelfäden.

3. Schlauch nach Anspruch 1, umfassend etwa ein Kettgarn für jeweils 2 elastische Litzen.

4. Schlauch nach Anspruch 3, worin die Einzelfäden ein Polyester sind.

5. Schlauch nach Anspruch 4, worin die Einzelfäden einen Durchmesser von 0,15 bis 0,375 mm (6 mils bis 15 mils) aufweisen.

6. Geflochtene Struktur nach Anspruch 5, worin die elastische Litze etwa 2 bis etwa 6 Kettfäden des Polyestereinzelfadens mit einem Durchmesser von etwa 0,15 bis 0,375 mm (6 bis etwa 15 mils) und einen Elastizitätsmodul von etwa 5171 MN/m² (7500.000 psi) umfaßt.

## Revendications

1. Gaine tubulaire flexible pouvant être installée in-situ comprenant des torons élastiques tressés, dans lequel chaque toron élastique est composé de 1 à 10 monofilaments d'un plastique technique ayant un module d'élasticité d'au moins 3447 MN/m² (500 000 psi), lesdits torons élastiques tressés définissant une pluralité de paires de points de croisement au sein de ladite gaine, ladite gaine tressée comprenant en outre des fils de chaîne relativement souples, flexibles et sensiblement non élastiques, répartis uniformément, entrelacés dans ladite tresse, ladite gaine ayant au moins une première et une seconde positions, de sorte que :
une portion desdits torons élastiques tressés dans ladite première position soit comprimée longitudinalement et dilatée radialement et lesdits fils de chaîne souples aient tendance à former uniformément de très petites boucles entre les paires de points de croisement où lesdits fils de chaîne sont situés dans ladite portion comprimée longitudinalement et dilatée radialement desdits torons élastiques tressés; et
dans ladite seconde position, ladite portion des torons élastiques tressés soit dilatée longitudinalement et comprimée radialement, et lesdits fils de chaîne souples soient sensiblement droits afin de rétracter sensiblement lesdites boucles.

2. Gaine selon la revendication 1, comprenant un fil de chaîne pour 1 à 4 monofilaments.

3. Gaine selon la revendication 1, comprenant un fil de chaîne pour 2 torons élastiques.

4. Gaine selon la revendication 3, dans laquelle les monofilaments sont en polyester.

5. Gaine selon la revendication 4, dans laquelle les monofilaments ont un diamètre de 0,15 à 0,375 mm (6 à 15 millièmes de pouce).

6. Structure tressée selon la revendication 5, dans laquelle ledit toron élastique comprend de 2 à 6 extrémités de monofilament de polyester ayant un diamètre de 0,15 à 0,375 mm (6 à 15 millièmes de pouce) et un module d'élasticité d'environ 5171 MN/m² (750 000 psi).
